

## UNITED STATES PATENT OFFICE

2,380,566

METHOD OF CONDITIONING MOLTEN Be-  
CONTAINING ALLOYS FOR CASTING

Francis O'Neill Wyllie, Reading, Pa., assignor, by  
mesne assignments, to Berks County Trust  
Company, Reading, Pa., a banking institution  
of Pennsylvania

No Drawing. Application December 13, 1941,  
Serial No. 422,876

5 Claims. (Cl. 75—76)

This invention relates to metallurgy and more particularly to the metallurgy of beryllium-copper alloys and has for its object the provision of an effective method of eliminating gases and undissolved occluded matter from molten beryllium-copper alloys.

Another object is to provide an effective method of purifying molten beryllium-copper alloys.

Still another object is to provide a method of conditioning molten beryllium-copper alloys for casting into sound ingots.

Other objects and advantages will be apparent as the invention is hereinafter more fully disclosed.

In accordance with these objects I have discovered that, contrary to expectations, molten beryllium-copper alloys may be completely degasified and freed of undissolved occluded matter by super-heating the alloys to temperatures within the range 1900°—2400° F., depending on the Be content and melting point of the Be-containing alloy being treated, blowing oxygen therethrough, and then deoxidizing the melt before the temperature of the melt falls to a temperature below about 1900° F., without occasioning any appreciable loss of beryllium in the alloy. By the term "super-heating" is meant heating to temperatures materially above the melting point of the alloy which varies with respect to the Be-content as one skilled in the art will recognize.

In the manufacture of beryllium-copper alloys, particularly the low beryllium content alloys containing beryllium within the range .3 to 3.0% it is exceedingly difficult to obtain a gas and occlusion-free cast ingot suitable for mechanical reduction to sheet, bar, rod and wire sizes. The usual foundry practices applied to copper alloys generally to eliminate gases and occlusions are not applicable to beryllium-containing copper alloys and usually result in material losses of beryllium. In accordance with the present invention, however, even extremely dirty and gassy metal may be quickly and effectively freed of dross and other suspended or occluded undissolved impurities and completely degasified and placed in condition for casting into sound workable ingots.

As an example of the present invention, the beryllium-copper alloy to be treated by the present invention is brought to the molten condition in a covered crucible in a reducing or neutral atmosphere as is customary in the art. The molten alloy is then super-heated to a temperature within the range 1900°—2400° F., and with the furnace heat turned off, substantially pure dry oxygen is blown through the molten metal at such a rate

as to vigorously agitate the super-heated molten metal. The oxygen blow is continued for an extended time interval while the temperature of the molten metal falls and is terminated before the temperature of the molten metal drops to a temperature approximating 1900° F.

The dross and insoluble material over the surface of the molten metal is then quickly skimmed off and a sufficient amount of a deoxidizer agent consisting at least in part of an alkali or alkaline earth metal, such as lithium-copper or calcium boride, is added to the molten alloy to effect a removal of the oxygen and metal oxides present in the molten metal. The molten metal is allowed to remain quiescent for a time interval to permit deoxidation to proceed to completion and if a trial casting indicates the metal is ready for casting the temperature of the molten and purified beryllium-copper alloy is adjusted to the desired casting temperature and the metal is poured.

The method above described is particularly adapted for use with molten beryllium-copper alloys made up at least in part from re-melted scrap material and is also of particular utility in the forming of beryllium-copper alloys from copper and beryllium-copper master alloy. In the forming of beryllium-copper alloys by the general method of diluting a beryllium-copper master alloy with copper until the desired beryllium content is obtained, considerable difficulty is experienced in eliminating dross and non-metallic occlusions from the molten metal. Where the master alloy has been prepared by the arc-furnace method described and claimed in Gahagan Patent No. 2,193,482, dated March 12, 1940, which patent is assigned to the same assignee as the present application, the master alloy frequently contains beryllium carbide, nitride and oxide occlusions as well as dross and substantially inert material such as silica sand. The copper employed in diluting the master alloy frequently contains large amounts of copper oxide and gases, such as hydrogen.

When substantially pure dry oxygen is passed through beryllium-copper alloys at temperatures above about 1900° F., the beryllium content of the alloy, particularly in the presence of hydrogen dissolved in the metal, appears substantially unaffected by the oxygen, the reaction appearing to go in the direction to form H·OH rather than in the direction to form BeO. At temperatures below 1900° F., however, the reaction appears to be reversed and the beryllium losses incident to oxidation are relatively high.

Having hereinabove described the present in-

vention generically and specifically and given one specific embodiment of the same it is believed apparent that the same may be widely varied without essential departure therefrom and all such modifications and departures are contemplated as may fall within the scope of the following claims.

What I claim is:

1. The method of preparing molten beryllium-copper alloys for casting which comprises heating the molten metal to temperatures materially above the melting point of the alloy, blowing the molten metal with oxygen for a time interval at least sufficient to eliminate therefrom substantially all of the hydrogen content thereof, maintaining the alloy throughout the oxygen blow at a temperature in excess of about 1900° F., and de-oxidizing the blown molten metal with a deoxidizer agent comprised at least in part of a metal of the group consisting of the alkali and alkaline earth metals before casting and solidifying the alloy.

2. In the melting and casting of copper alloys containing beryllium as one alloy constituent, the method of conditioning the molten alloy for casting which comprises super-heating the molten alloy to a temperature within the range 1900°-2400° F., blowing oxygen through the super-heated alloy for a time interval at least sufficient to remove substantially all of the hydrogen content thereof and to bring to the surface of the alloy substantially all of the dross and undissolved foreign matter suspended therethrough, and then deoxidizing the alloy with a deoxidizer agent com-

prised at least in part of a metal of the alkali metal and alkaline earth metal groups.

3. The method of claim 2, wherein the temperature of the molten alloy is maintained at a temperature above about 1900° F., during the oxygen blow therethrough.

4. The method of degasifying molten beryllium-containing copper alloys which comprises heating the alloy to temperatures above about 1900° F., blowing oxygen through the molten alloy for a time interval at least sufficient to eliminate the hydrogen content of the alloy and to provide a slight excess of dissolved oxygen in the alloy, and then deoxidizing the molten alloy by appropriate additions of a metal of the alkali and alkaline earth metal group.

5. The method of conditioning molten beryllium-containing copper alloys for casting which comprises super-heating the alloy to temperatures within the range 1900°-2400° F., blowing oxygen gas therethrough while maintaining a temperature above about 1900° F., for an extended time interval at least sufficient to provide for the collection of substantially all of the occluded insoluble and non-oxidizable impurities of the metal into a surface dross and for the oxidation of substantially all of the occluded insoluble and oxidizable impurities of the metal into a surface dross and for the oxidation of substantially all hydrogen contained in the molten metal, removing the surface dross and deoxidizing the molten metal bath with appropriate additions of a metal of the alkali and alkaline earth metal groups before casting.

FRANCIS O'NEILL WYLLIE.